

# UNITED STATES PATENT OFFICE.

WILLIAM H. ALLEN, OF DETROIT, MICHIGAN, ASSIGNOR TO PARKER RUST-ROOF COMPANY, OF DETROIT, MICHIGAN, A CORPORATION OF MICHIGAN.

## PROCESS FOR CONTROLLING CASE-HARDENING.

1,377,174.

Specification of Letters Patent.

Patented May 10, 1921.

No Drawing. Application filed April 17, 1919, Serial No. 290,748. Renewed January 17, 1921. Serial No. 437,968.

*To all whom it may concern:*

Be it known that I, WILLIAM H. ALLEN, a citizen of the United States, and residing at Detroit, in the county of Wayne and State 5 of Michigan, have invented new and Improved Processes for Controlling Case-Hardening, of which the following is a specification.

It has long been known that the area of 10 carbonization or case-hardening of an article of iron or steel may be limited by copper-plating such surfaces as are to remain soft before subjecting the article to the action of the carbonizing gases in the cementation or case-hardening chamber or receptacle.

It has also been known for some time that 20 in order to perfectly "rust-proof" articles of iron and steel by the processes set forth in the patents granted to Coslett, No. 870,937, dated November 12, 1907, and to Richards, No. 1,069,903, dated August 12, 1913, that the metal must be clean in order to permit proper action by the solution of ferric phosphate.

When the surfaces of articles of iron and steel have been changed from metallic iron to ferro-ferric phosphate by the "rust-proofing" processes described in the above 30 named patents, cementation or case-hardening action is retarded, and when the "rust-proofing" process is imperfect, the case-hardening gases have effect. I have discovered that when the articles are covered in 35 whole or in part with an organic substance that is insoluble in aqueous slightly acid solutions, such as shellac and other varnishes, that the "rust-proofing" process described in said patents has no effect on such coated 40 areas.

I have further discovered that when a "rust-proofed" surface is coated with a thin film of fused acid phosphates of sodium or potassium, or other salts, such as borax or 45 borate of ammonia and soluble silicates, as are fusible at about the temperature within the case-hardening chamber, that the case-hardening action is entirely prevented for such "rust-proofed" areas. It appears that 50 the fused salt enters the minute interstices of the ferro-ferric phosphate surface and seals them, preventing the entrance of the gases of the cementation process.

I have also discovered that where certain areas of articles of iron and steel are coated 55 with shellac or other readily fusible organic material and the articles are "rust-proofed," that when these articles are treated by the case-hardening process that the areas that were coated become case-hardened. 60

My present process consists in coating such surfaces of articles of iron and steel as are to be case-hardened with an organic substance, such as varnish, which is insoluble in the "rust-proofing bath, then treating 65 the articles so as to change the non-coated surfaces from metallic iron to iron phosphates, and then subjecting these articles to the case-hardening process, with or without the intermediate step of coating the 70 iron phosphate surfaces with a film of fused inorganic salt.

I claim:—

1. The process of hardening selected areas 75 of articles of iron and steel which consists in coating such areas with a material which may be disintegrated by heat but is insoluble in aqueous slightly acid solutions, changing the remaining areas from metallic iron to iron phosphates, and then subjecting the 80 articles to the action of case-hardening gases.

2. The process of hardening selected areas 85 of articles of iron and steel which consists in coating such areas with varnish, changing the remaining areas from metallic iron to iron phosphates, and then subjecting the 90 articles to the action of case-hardening gases.

3. The process of hardening selected areas 95 of articles of iron and steel which consists in coating such areas with a material which may be disintegrated by heat but is insoluble in aqueous slightly acid solutions, changing, the remaining areas from metallic iron to iron phosphates, coating the 100 article with fused salts, and then subjecting the articles to the action of case-hardening gases.

4. The process of hardening selected areas 105 of articles of iron and steel which consists in coating such areas with shellac, changing the remaining areas to iron phosphates, coating the articles with fused sodium phosphate, and then subjecting the articles to the action of case-hardening gases.

WILLIAM H. ALLEN.